

July 13, 1971

C. M. BROWN ET AL

3,592,637

METHOD FOR ADDING METAL TO MOLTEN METAL BATHS

Filed Feb. 26, 1968



**INVENTORS**

CHARLES M. BROWN

NICHOLAS J. PAPPAS

HARRY J. BROWN

BY

*Frank J. McCloskey*  
ATTORNEY

1

3,592,637

METHOD FOR ADDING METAL TO  
MOLTEN METAL BATHS

Charles M. Brown, Lewiston, Nicholas J. Pappas, Snyder,  
and Harry J. Brown, Lewiston, N.Y., assignors to  
Union Carbide Corporation  
Filed Feb. 26, 1968, Ser. No. 708,267  
Int. Cl. C22c 1/02

U.S. Cl. 75—138

11 Claims

ABSTRACT OF THE DISCLOSURE

A method of addition of a metal to a molten metal bath by mixing the aluminum to be dissolved in finely divided form with a solution promoting aluminum, also in finely divided form, and adding the mixture to molten metal.

This invention relates to the addition of metallic materials to molten metal baths. More particularly, the present invention relates to addition agents formed of finely divided solid metal particles having improved solution rates in molten metal baths.

It is a common practice in metallurgical operations to provide an ultimate desired alloy composition by the introduction of solid metal additives to molten metal baths of a base metal. For example, manganese is added to molten aluminum in the form of manganese-aluminum alloy containing about 5-20% manganese, to provide increased strength in wrought aluminum products. Also, chromium, tungsten, molybdenum, vanadium, iron, cobalt, copper, nickel, columbium and other metals are commonly added in pre-alloyed form to molten metal baths to obtain a particular alloy product. Chromium, for example, has been added to aluminum baths to provide improved corrosion resistance and molybdenum, iron, vanadium and chromium have been added to titanium as stabilizers.

The past practices however have almost universally employed relatively expensive pre-alloyed additions which did not have completely satisfactory solution rates and quite often result in large and highly undesirable temperature drops in the bath to which they are added.

It is therefore an object of the present invention to provide metal bearing addition agents which can be economically prepared and which can be effectively and advantageously added directly to molten metal baths.

Other objects will be apparent from the following description and claims taken in conjunction with the drawing which shows a graph illustrating exemplary solution rates for various addition agents, including particular additions in accordance with the present invention.

An addition agent in accordance with the present invention comprises a blended mixture of at least two different finely divided metal bearing materials in particular proportions whereby upon addition to a molten metal bath the metals rapidly dissolve with relatively little temperature drop being developed in the molten metal bath.

The addition agent of the present invention can be considered as comprising a "solution promoter" material and a "principal material"; the principal material being generally the metal, whose rapid solution is particularly desired.

In the present invention, the promoter materials include the following elements:

2

Al  
Si

and the principal materials include the following elements:

|       |    |    |
|-------|----|----|
| Mn    | V  | Cb |
| Cr    | Fe | Ta |
| W     | Co | Zr |
| Mo    | Cu | Hf |
| 10 Ti | Ni | Ag |

It has been found, as part of the present invention, that a principal material, when blended in finely divided form with a promoter material, in proportions as hereinafter described, can be dissolved in a metal bath at a remarkably increased rate due to coaction between the principal and promoter elements. Thus for example, a mixture of finely divided aluminum with finely divided manganese, in appropriate proportions, results in increased rate of manganese solution upon addition to a molten bath as compared to a Mn-Al alloy of the same proportions. Similarly, the principal material chromium can be blended with the promoter aluminum to provide increased rate of solution for chromium. That is to say, the solution of any principal material, when blended in finely divided form with any promoter, in accordance with the present invention, will be significantly improved.

In addition to the elemental metals listed above the promoter material can be in the form of an alloy containing at least 50% by weight in the aggregate of promoter elements and in which the aggregate of the principal elements does not exceed a certain value as herein-after defined.

Correspondingly, the principal material can be an alloy containing at least 50% by weight principal elements and in which the aggregate of alloyed promoter elements is not more than a specified amount also as herein-after defined.

An important aspect of the present invention as regards solution rate and bath temperature drop is that the relationships of uncombined (i.e. unalloyed) principal material to uncombined promoter material must be within certain limits. These relationships, designated (A), (B) and (C) hereinbelow, are expressed as follows:

(A)

Broad:

$$9 \geq \frac{\text{Percent Effective Principal Material} \times K_1}{\text{Percent Effective Promoter Material} \times K_2} \geq 0.11$$

50 Preferred:

$$2.33 \geq \frac{\text{Percent Effective Principal Material} \times K_1}{\text{Percent Effective Promoter Material} \times K_2} \geq 0.428$$

(B)

Percent Effective Principal Material  $\geq 20$ ; preferably  $\geq 30$

(C)

60 Percent Effective Principal Material  $\geq 20$ ; preferably  $\geq 30$   
where

K<sub>1</sub>=The aggregate amount by weight of principal material in the addition agent.

65 K<sub>2</sub>=The aggregate amount by weight of promoter material in the addition agent.

PERCENT EFFECTIVE PRINCIPAL MATERIAL =  $\Sigma$  IN THE PRINCIPAL MATERIAL OF —

|                   |                                                                   |          |                                                                                                                                        |
|-------------------|-------------------------------------------------------------------|----------|----------------------------------------------------------------------------------------------------------------------------------------|
| Percent Mn =      | $\frac{\text{Wt. of Mn}}{\text{Total wt. of principal elements}}$ | $\times$ | Percent of alloyed Al in the principal material plus $2 \times$ the percent of alloyed Si in the principal material.                   |
| Plus percent Ti = | $\frac{\text{Wt. of Ti}}{\text{Total wt. of principal elements}}$ | $\times$ | $1.25 \times$ the percent of alloyed Al in the principal material plus $3 \times$ the percent of alloyed Si in the principal material. |
| Plus percent V =  | $\frac{\text{Wt. of V}}{\text{Total wt. of principal elements}}$  | $\times$ | $0.66 \times$ percent of alloyed Al in the principal material plus $3 \times$ the percent of alloyed Si in the principal material.     |
| Plus percent Mo = | $\frac{\text{Wt. of Mo}}{\text{Total wt. of principal elements}}$ | $\times$ | $1.25 \times$ percent of alloyed Al in the principal material plus $2 \times$ the percent of alloyed Si in the principal material.     |
| Plus percent W =  | $\frac{\text{Wt. of W}}{\text{Total wt. of principal elements}}$  | $\times$ | $1.25 \times$ percent of alloyed Al in the principal material plus $10 \times$ the percent of alloyed Si in the principal material.    |
| Plus percent Co = | $\frac{\text{Wt. of Co}}{\text{Total wt. of principal elements}}$ | $\times$ | $2 \times$ percent of alloyed Al in the principal material plus $2 \times$ the percent of alloyed Si in the principal material.        |
| Plus percent Fe = | $\frac{\text{Wt. of Fe}}{\text{Total wt. of principal elements}}$ | $\times$ | $0.66 \times$ percent of alloyed Al in the principal material plus $2 \times$ the percent of alloyed Si in the principal material.     |
| Plus percent Cr = | $\frac{\text{Wt. of Cr}}{\text{Total wt. of principal elements}}$ | $\times$ | $2 \times$ percent of alloyed Al in the principal material plus $2 \times$ the percent of alloyed Si in the principal material.        |
| Plus percent Ni = | $\frac{\text{Wt. of Ni}}{\text{Total wt. of principal elements}}$ | $\times$ | $2 \times$ percent of alloyed Al in the principal material plus $2 \times$ the percent of alloyed Si in the principal material.        |
| Plus percent Zr = | $\frac{\text{Wt. of Zr}}{\text{Total wt. of principal elements}}$ | $\times$ | $2 \times$ percent of alloyed Al in the principal material plus $3 \times$ the percent of alloyed Si in the principal material.        |
| Plus percent Cu = | $\frac{\text{Wt. of Cu}}{\text{Total wt. of principal elements}}$ | $\times$ | $4 \times$ percent of alloyed Al in the principal material plus $15 \times$ the percent of alloyed Si in the principal material.       |
| Plus percent Hf = | $\frac{\text{Wt. of Hf}}{\text{Total wt. of principal elements}}$ | $\times$ | $4 \times$ percent of alloyed Al in the principal material plus $3 \times$ the percent of alloyed Si in the principal material.        |
| Plus percent Ag = | $\frac{\text{Wt. of Ag}}{\text{Total wt. of principal elements}}$ | $\times$ | $11 \times$ percent of alloyed Al in the principal material plus $2 \times$ the percent of alloyed Si in the principal material.       |
| Plus percent Cb = | $\frac{\text{Wt. of Cb}}{\text{Total wt. of principal elements}}$ | $\times$ | $10 \times$ percent of alloyed Al in the principal material plus $5 \times$ the percent of alloyed Si in the principal material.       |
| Plus percent Ta = | $\frac{\text{Wt. of Ta}}{\text{Total wt. of principal elements}}$ | $\times$ | $19 \times$ percent of alloyed Al in the principal material plus $3 \times$ the percent of alloyed Si in the principal material.       |

and where

PERCENT EFFECTIVE PROMOTER MATERIAL =  $\Sigma$  IN THE PROMOTER MATERIAL OF -

|                                                                                               |                                                                                                                                                                                                                                                                                                                                                                                                                                                                                                                                                                                                                                                                                                                                                                                                                                                                                                                                                                         |
|-----------------------------------------------------------------------------------------------|-------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------|
| $\text{Percent Al} = c \times \frac{\text{Wt. of Al}}{\text{Total wt. of promoter elements}}$ | Percent of alloyed Mn in the promoter material.<br>Plus $0.8X$ percent of alloyed Ti in the promoter material.<br>Plus $0.8X$ percent of alloyed Mo in the promoter material.<br>Plus $0.8X$ percent of alloyed W in the promoter material.<br>Plus $1.5X$ percent of alloyed V in the promoter material.<br>Plus $0.45X$ percent of alloyed Co in the promoter material.<br>Plus $0.45X$ percent of alloyed Cr in the promoter material.<br>Plus $0.45X$ percent of alloyed Ni in the promoter material.<br>Plus $0.45X$ percent of alloyed Zr in the promoter material.<br>Plus $0.25X$ percent of alloyed Cu in the promoter material.<br>Plus $0.25X$ percent of alloyed Hf in the promoter material.<br>Plus $0.09X$ percent of alloyed Ag in the promoter material.<br>Plus $0.1X$ percent of alloyed Cb in the promoter material.<br>Plus $0.05X$ percent of alloyed Ta in the promoter material.<br>Plus $1.5X$ percent of alloyed Fe in the promoter material. |
|-----------------------------------------------------------------------------------------------|-------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------|

Plus:

|              |                                |                                                            |
|--------------|--------------------------------|------------------------------------------------------------|
| Percent Si = | Wt. of Si                      | Plus 0.5X percent of alloyed Mn in the promoter material.  |
|              | Total wt. of promoter elements | Plus 0.33X percent of alloyed Ti in the promoter material. |
|              |                                | Plus 0.33X percent of alloyed V in the promoter material.  |
|              |                                | Plus 0.33X percent of alloyed Mo in the promoter material. |
|              |                                | Plus 0.1X percent of alloyed W in the promoter material.   |
|              |                                | Plus 0.5X percent of alloyed Co in the promoter material.  |
|              |                                | Plus 0.5X percent of alloyed Fe in the promoter material.  |
|              |                                | Plus 0.5X percent of alloyed Cr in the promoter material.  |
|              |                                | Plus 0.5X percent of alloyed Ni in the promoter material.  |
|              |                                | Plus 0.33X percent of alloyed Zr in the promoter material. |
|              |                                | Plus 0.06X percent of alloyed Cu in the promoter material. |
|              |                                | Plus 0.33X percent of alloyed Hf in the promoter material. |
|              |                                | Plus 0.5X percent of alloyed Ag in the promoter material.  |
|              |                                | Plus 0.2X percent of alloyed Cb in the promoter material.  |
|              |                                | Plus 0.33X percent of alloyed Ta in the promoter material. |

The foregoing relationships have been discovered as a result of extensive testing and study of the principal and promoter materials.

The relationship (A) as defined above in general represents the overall balance between "free" or "active" principal and promoter materials that is required in an addition agent for effective coaction, while relationships (B) and (C) define the amount of "free" or "active" principal and promoter elements required, in the principal and promoter materials respectively, for effective coaction and improved solution properties. Relationship (B) shows that only materials containing more than a defined amount of "free," i.e. uncombined, unalloyed principal material are suitable, i.e. active enough to function as principal materials, and relationship (C) provides a corresponding relationship for the promoter materials. The definitions "Percent Effective Principal Material" and "Percent Effective Promoter Material" further show that the permissible extent of alloying depends upon the particular principal and promoter elements involved. For example, an alloy of 60% Mn, 40% Al will be suitable as a principal material since the Percent Effective Principal Material in such an alloy is  $60-40=20$ . However, an alloy of 60% Mn, 40% Si alloy on account of the different interaction between manganese and silicon would not be a suitable principal material and the Percent Effective Principal Material in such an alloy is  $60-2\times40=-20$  which is not  $\geq 20$ . An alloy of about 73.5% Mn, 26.5% Si would however be a suitable principal material. As to promoter materials, an alloy of 60% Al, 40% Mn will be a suitable promoter material since the Percent Effective Promoter Material would be  $60-40=20$ . An alloy of 60% Al, 40% V however would not be suitable as a promoter material since the Percent Effective Promoter Material in such a case would be  $60-1.5\times40=0$ . Further with respect to the aforementioned relationships (A), (B) and (C), in the more complex addition agents it must be kept in mind that all materials qualifying as principal materials are "lumped together" for purposes of computing percentages and factors applicable to the Percent Effective Principal Material, and all materials qualifying as promoter materials are "lumped together" for purposes of computing percentages and factors applicable to the Percent Effective Promoter Material.

The following Examples A through I are given to further illustrate how the foregoing relationships are calculated for specific addition agents.

In the case where interalloying of principal and promoter material is not present in the addition agent rela-

tionships (B) and (C) can be ignored (both the Percent Effective Principal Material and the Percent Effective Promoter Material=100); also, relationship (A) in this case is:

30 Broad: 10 to 90% Principal Material and 10 to 90% Promoter Material  
Preferred: 20 to 80% Principal Material and 20 to 80% Promoter Material

35

#### EXAMPLE A

The addition agent is a mixture of 60 parts by weight of finely divided aluminum and 40 parts by weight of finely divided manganese.

40  $K_1=40$   
 $K_2=60$

Percent Effective Principal Material (B)=100 (Mn constitutes 100% of the principal material)  
Percent Effective Promoter Material (C)=100 (Al constitutes 100% of the promoter material)

thus (A) is

$$50 \quad \frac{40\times100}{60\times100}=0.67$$

#### EXAMPLE B

55 The addition agent is a mixture of 60 parts by weight of 80% Mn-20% Al alloy and 40 parts by weight of finely divided elemental aluminum.

56  $K_1=60$   
 $K_2=40$

Percent Effective Principal Material (B) =  $80 - \frac{48}{48} \times 20 = 60$   
Percent Effective Promoter Material (C) =  $100$  (Al constitutes 100% of the promoter material)

65 thus (A) is  $\frac{60\times60}{40\times100}=0.9$

70

#### EXAMPLE C

The addition agent is a mixture of 50 parts by weight of 80% Al-20% Si alloy and 50 parts by weight of 95% Mn-5% Al alloy.

75

$K_1=50$  (parts of the principal material: 95% Mn-5% Al alloy)

$K_2=50$  (parts of the promoter material: 80% Al-20% Si)

$$\text{Percent Effective Principal Material} = 95 - \frac{47.5}{47.5} \times 5 = 90$$

Percent Effective Promoter Material

$$= 80 - \frac{40}{50} \times 0 + 20 - \frac{10}{50} \times (0) = 100$$

$$\text{thus (A) is } \frac{50 \times 90}{50 \times 100} = 0.9$$

$K_1=60$  (40 parts of Mn+20 parts of 80% Mn-20% Al)

$K_2=40$  (40 parts of aluminum)

$$\text{Percent Effective Principal Material (B)} = 93\% - \frac{56}{56} (6.7\%) = 86.3$$

$$\text{Percent Effective Promoter Material (C)} = 100$$

$$\text{thus (A) is } \frac{86.3 \times 60}{100 \times 40} = 1.3$$

#### EXAMPLE H

The addition agent is a mixture of 200 parts of 50% Mn-20% Ti-20% Al-10% Si alloy and 200 parts of elemental aluminum.

15

$K_1=200$

$K_2=200$

$$\text{Percent Effective Principal Material} = 50 - \frac{100}{140} \times (20 + 2 \times 10) = 20 - \frac{40}{140} (1.25 \times 20 + 3 \times 10) = 21.4 + 4.3 = 25.7$$

25

$$\text{Percent Effective Promoter Material} = 100$$

$$\text{thus (A) is } \frac{25.7 \times 200}{100 \times 200} = 0.257$$

30

#### EXAMPLE I

The addition agent is a mixture of 50 parts of elemental manganese, 50 parts of 40% Ti-40% Al-20% Si alloy, and 100 parts of elemental aluminum. (Note: The Ti-Al-Si alloy is a promoter material since Al+Si>50%.)

35

$K_1=50$

$K_2=150$

$$\text{Percent Effective Principal Material} = 100$$

Percent Effective Promoter Material:

$$\text{Percent Al} = 100 \text{ parts of elemental Al} + 40\% \text{ of 50 parts of Al containing alloy} \div 150 \text{ parts of total Promoter Material} = 80\%$$

45

$$\text{Percent Si} = 20\% \text{ of 50 parts of Si containing alloy} \div 150 \text{ parts of total Promoter Material} = 6.67\%$$

$$\text{Percent Ti alloyed in Promoter Material} = 40\% \text{ of 50 parts of Ti-containing alloy} \div 150^* \text{ parts of total Promoter Material} = 13.3\%$$

50

Percent Effective Promoter

$$= 80 - \frac{120}{100 + 20 + 10} (0.8 \times 13.3)$$

$$+ 6.67 - \frac{10}{100 + 20 + 10} (0.33 \times 13.3) = 76.51$$

55

$$\text{thus (A) is } \frac{100 \times 50}{76.51 \times 150} = 0.44$$

60

To further illustrate the present invention, the following Tables I(a) and I(b) list various other specific promoter and principal materials, which are effective in the practice of the present invention.

65

#### Table I(a).—Specific promoter materials (alloys)

70% Al, 30% V

80% Al, 20% Ti

70% Al, 20% Mn

75% Si, 25% Fe

70% Si, 5% Mg, bal Fe

60-65% Si, 1% Al, 6% Zr, 2% Ca, 3% Ba, bal Fe

75

\*50 parts of Ti-Al-Si alloy + 100 parts of Al.

#### EXAMPLE F

The addition agent is a mixture of 40 parts by weight of finely divided 95% Mn-5% Al alloy and 20 parts by weight of finely divided 70% Al-30% Mn alloy.

$K_1=80$

$K_2=20$

$$\text{Percent Effective Principal Material (B)} = 95 - \frac{95}{95} \times 5 = 90$$

$$\text{Percent Effective Promoter Material (C)} = 70 - \frac{70}{70} \times 30 = 40$$

$$\text{thus (A) is } \frac{90 \times 80}{40 \times 20} = 9$$

$K_1=60$  (40 parts of Mn+20 parts of 80% V-20% Al)

$K_2=40$  (40 parts of aluminum)

Percent Effective Principal Material (B)

$$= 67\% - \frac{40}{56} \times 6.7\% + 26.6\% - \frac{16}{56} (0.66 \times 6.7) = 87.7$$

Percent Effective Promoter Material (C) = 100 (all of promoter is aluminum)

$$\text{thus (A) is } \frac{87.7 \times 60}{100 \times 40} = 1.32$$

#### EXAMPLE G

The addition agent is a mixture of 40 parts by weight of finely divided manganese, 20 parts by weight of finely divided 80% Mn-20% Al alloy and 40 parts by weight of finely divided aluminum.

Table I(b).—Specific principal materials (alloys)

|                                 |
|---------------------------------|
| 90% W, 10% Al                   |
| 80% W, 20% Fe                   |
| Nitrided manganese (up to 8% N) |
| 93% Mn, 2% Si, 1.8% C, bal Fe   |
| 70% Cr, 2% Si, bal Fe           |
| 85% V, 15% Al                   |
| 70% V, 30% Fe                   |
| 67% Ti, bal Fe                  |
| 60% Mn, 40% Cu                  |

As to the physical form of the addition agent of the present invention, it can be used as an uncompacted confined mixture, for example, the mixture of principal and promoter material can be wrapped in metal foil or enclosed in consumable containers. When used in such form it is introduced beneath the surface of the molten bath by customary plunging or immersion devices and techniques. Most often and preferably however the addition agent of this invention is employed in the form of pressed compacts or pellets which preferably have sufficient density so that they sink of their own weight in the molten metal bath. In either case, the initial sizing of the constituent promoter and principal materials is important and should be substantially all finer than 20 mesh for optimum solubility and preferably substantially all finer than 65

—0.039 which is referred to herein as the solution rate K. The procedure of this example was followed with other additions to obtain their solution rates and these are listed herein below. Increasing numerical values for K, i.e. more negative values, represent more rapid solution rates.

## EXAMPLE 2

The procedure of Example 1 was followed using 34 gram pellets (7/8 inch diameter) formed by pressing 10 blended mixtures of materials selected from those listed in Table II(a) at 20,000 p.s.i. in a hydraulic press. The pellets had the densities indicated in Table II(b) which also shows the solution rates obtained.

TABLE II(a)

|    | Material                  | Composition                     | Initial sizing              |
|----|---------------------------|---------------------------------|-----------------------------|
| 15 | Manganese flake           | 100% Mn                         | 150 mesh and finer (150XD). |
|    | Aluminum                  | 100% Al                         | —100 mesh—325 mesh.         |
| 20 | LoFe ferromanganese       | 90% Mn, 2% Si, 6.7% C, bal. Fe  | 65 mesh and finer (65XD).   |
|    | LoSi, LoFe ferromanganese | 86% Mn, 9% Si, 0.05% C, bal. Fe | Do.                         |

Other materials, including a commercial manganese containing addition agent (5% Mn "hardener"—bal. Al) 25 were also tested following the procedure of Example 1 and the results are shown in Table II(b) for purposes of comparison:

TABLE II(b)

| Bath temp., °C.                            |  | Rate of solution, K |        | Percent theor. | Mn recovery, percent |
|--------------------------------------------|--|---------------------|--------|----------------|----------------------|
|                                            |  | 760                 | 850    |                |                      |
| Form of addition, sample:                  |  |                     |        |                |                      |
| P-1 (5% Mn+95% Al) <sup>1</sup>            |  | —0.032              |        | 2.41           | 86 95+               |
| P-2 (20% Mn+80% Al) <sup>2</sup>           |  | —0.50               |        | 2.56           | 83 95+               |
| P-3 (50% Mn+50% Al) <sup>2</sup>           |  | —0.55               |        | 3.53           | 88 95+               |
| P-4 (90% Mn+10% Al) <sup>2</sup>           |  | —0.20               |        | 4.26           | 68 95+               |
| 5 (LoFe, FeMn) 8XD                         |  |                     | —0.005 |                | 95+                  |
| P-6 (50% LoFeFeMn+50% Al) <sup>2</sup>     |  | —0.75               | 3.16   | 64             | 95+                  |
| 7 (5% Mn "hardener" 1/2" lumps)            |  | —0.152              | —0.18  |                | 95+                  |
| 8 Mn flake 2" x 1/2" lumps                 |  | —0.019              | —0.039 |                | 95+                  |
| 9 Mn flake 1/2"                            |  | —0.024              | —0.047 |                | 95+                  |
| 10 Mn flake 20 mesh                        |  | —0.074              | —0.131 |                | 95+                  |
| 11 Mn flake 150 mesh                       |  | —0.266              |        |                | 95+                  |
| 12 LoFe, FeMn 3/4" lumps                   |  |                     | —0.005 |                | 95+                  |
| 13 60% Mn, 40% Al (alloy) 3/4"             |  | —0.122              | —0.235 |                | 95+                  |
| 14 LoSi, LoFe, FeMn —SM+20M                |  | —0.018              |        |                | 95+                  |
| P-15 LoSi, LoFe, FeMn +50% Al <sup>2</sup> |  | —0.60               | 3.53   |                | 95+                  |

<sup>1</sup> P represents pellet addition.

<sup>2</sup> This invention.

mesh. The principal and promoter materials preferably constitute at least 80% by weight of the addition.

When pressed mixtures are employed it has been found that very high compact densities should be avoided to obtain best solution rates. Densities above 95% of the maximum theoretical density (the maximum theoretical density being that of the melted fully alloyed constituents) should be avoided.

To more particularly illustrate the present invention various tests were performed and the data obtained is shown in the following examples.

## EXAMPLE 1

A bath of molten aluminum (5 lbs.) was stabilized at 850° C. and a 1.5% addition (34 grams) of manganese was added as electrolytic manganese flake (2" x 1/8" lumps). At the various time increments listed below samples were taken from the bath and analyzed for manganese:

| Time from addition, minutes | Actual analysis, percent Mn dissolved | Percent Mn undissolved (by subtraction) |
|-----------------------------|---------------------------------------|-----------------------------------------|
| Base:                       |                                       |                                         |
| t=0                         | 0.02                                  | 1.5                                     |
| t=2                         | 0.28                                  | 1.24                                    |
| t=4                         | 0.50                                  | 1.02                                    |
| t=8                         | 0.84                                  | 0.68                                    |
| t=15                        | 1.12                                  | 0.40                                    |

The foregoing data plotted conventionally on semi-log coordinates as shown in the drawing gives a slope of

As can be seen from the data of Table II(b), the addition agents in accordance with the present invention have very fast solution rates, i.e. more negative values for K. In particular it can be seen that additions P-2, P-3, P-6 50 and P-15 of this invention have solution rates several times faster than that of the "commercial hardener" addition 7 and the fully alloyed 60% Mn-40% Al addition 13. The solution rates for P-3 and the "commercial hardener" are comparatively illustrated in the drawing.

As shown in Table II(b), addition agents of the present invention containing about 50% Mn+50% Al (P-3 and P-6) have remarkably fast solution rates. Thus addition agents containing substantially equal amounts and percentages of Effective Principal Material and Effective Promoter Material are preferred. It will be noted that the 150 mesh electrolytic manganese addition 11 provides a respectable solution rate. However, manganese in this form is not practical as a commercial addition agent for aluminum since it would not readily penetrate the dross which develops on the top of an aluminum bath, oxidation losses of manganese would be considerable, and there would be problems of pyrophority and dusting.

Additional tests were performed to demonstrate the improved principal material solubility rate obtained through 70 the practice of the present invention as illustrated in the following examples.

## EXAMPLE 3

Pellets (7/8 inch diameter) were made by pressing tungsten powder (7 microns) at 5 ton p.s.i. pressure. 75 Pellets thus prepared were added to a molten aluminum

bath at 850° C. in an amount sufficient to provide a 1% tungsten addition. No detectable solution of tungsten was obtained.

#### EXAMPLE 4

Pellets (1/8 inch diameter) were made by pressing 50 parts by weight of tungsten powder (7 microns) with 50 parts by weight of aluminum powder (-100+325 mesh) at 5 ton p.s.i. pressure. Pellets (density=3.7 g./cc.) thus prepared were added to a molten aluminum bath at 760° C. in an amount sufficient to provide a 1% tungsten addition. The solution rate, K, obtained was -0.036. More than 95% of the added tungsten was dissolved.

#### EXAMPLE 5

Pellets (1/8 inch diameter) were made by pressing molybdenum powder (7 microns) at 5 ton p.s.i. pressure. Pellets thus prepared were added to a molten aluminum bath at 850° C. in an amount sufficient to provide a 1% molybdenum addition. No detectable solution of molybdenum was obtained.

#### EXAMPLE 6

Pellets (1/8 inch diameter) were made by pressing 50 parts by weight of molybdenum powder (7 microns) with 50 parts by weight of aluminum powder (-100+325 mesh) at 5 ton p.s.i. pressure. Pellets (density=3.3 g./cc.) thus prepared were added to a molten aluminum bath at 760° C. in an amount sufficient to provide a 1% molybdenum addition. The solution rate, K, obtained was -0.029. More than 95% of the added molybdenum was dissolved.

#### EXAMPLE 7

Ferrochromium (70% Cr, 2% Si, bal Fe) powder (150 mesh XD) was wrapped in metal foil and added to a molten aluminum bath at 760° C. in an amount sufficient to provide a 1 1/2% chromium addition. The solution rate, K, obtained was -0.002.

#### EXAMPLE 8

Pellets (1/8 inch diameter) were made by pressing 50 parts by weight of ferrochromium powder (150 mesh XD) with 50 parts by weight of aluminum powder (-100+325 mesh) at 5 ton p.s.i. pressure. Pellets (density=3.08 g./cc.) thus prepared were added to a molten aluminum bath at 760° C. in an amount sufficient to provide a 1 1/2% chromium addition. The solution rate, K, obtained was -0.093. More than 95% of the added chromium was dissolved.

#### EXAMPLE 9

Elemental chromium powder (150 XD) was wrapped in metal foil and added to a molten aluminum bath at 790° C. in an amount sufficient to provide a 3 1/2% chromium addition. The solution rate, K, obtained was -0.068.

#### EXAMPLE 10

Pellets (1/8 inch diameter) were made by pressing 50 parts by weight of elemental chromium powder (65 XD) with 50 parts by weight of aluminum powder (-100+325 M) at 5 ton p.s.i. pressure. Pellets (density=3.15 g./cc.) thus prepared were added to a molten aluminum bath at 760° C. in an amount sufficient to provide a 1 1/2% chromium addition. The solution rate, K, obtained was -0.56. More than 95% of the added chromium was dissolved.

#### EXAMPLE 11

Pellets (1/8 inch diameter) were made by pressing 50 parts by weight of 85% Mn-9% Si-bal Fe alloy powder (60 XD) with 42 parts by weight of 92% Al-8% Cr powder (65 XD) at 5 ton p.s.i. pressure. Pellets (density=3.21 g./cc.) thus prepared were added to a molten aluminum bath at 760° C. in an amount sufficient to

provide a 1 1/2% manganese addition. The solution rate, K, obtained was -0.14. More than 95% of the added manganese was dissolved.

#### EXAMPLE 12

Pellets (1/8 inch diameter) were made by pressing 37 parts by weight of manganese powder (150 XD) with 63 parts by weight of 60% Al-40% V alloy (65 XD) at 5 ton p.s.i. pressure. Pellets (density=2.65 g./cc.) thus prepared were added to a molten aluminum bath at 760° C. in an amount sufficient to provide a 1 1/2% manganese addition. The solution rate, K, obtained was -0.04.

In addition to the foregoing additional tests were conducted to determine the aluminum bath temperature drop for 1.5% Mn additions using a thermocouple immersed in the metal bath for temperature measurements. The results are shown in Table III.

TABLE III

Bath temperature drop for 1.5% Mn additions

|                                |                            | Temp. drop, ° C. |
|--------------------------------|----------------------------|------------------|
|                                | Bath temperature, ° C..... | 730 760          |
| Addition:                      |                            |                  |
| (7) "Commercial hardener"..... | 70                         | 90               |
| (P-3) 50% Mn+50% Al.....       | 8                          | 8                |

As can be seen, the addition agent of the present invention P-3 results in only a minor temperature drop as compared to the commercial material. The avoidance of bath-chilling by the user of the present invention is a very significant advantage in commercial operations.

Further tests were also conducted with compacted addition agents formed from electrolytic manganese and elemental aluminum prepared as described in Example II except that the densities of the compacts were varied to determine the effect of density on solution rate. The results are shown in Table IV.

TABLE IV

Effect of compact density on solution rate

|                          |     | Percent of max. density | Density, g./cc. | Solution rate, K, 760° C. bath temp. |
|--------------------------|-----|-------------------------|-----------------|--------------------------------------|
| Addition agent           |     |                         |                 |                                      |
| (P-3) 50% Mn+50% Al..... | 88  | 3.53                    | -0.55           |                                      |
| (P-3) 50% Mn+50% Al..... | 61  | 2.4                     | -0.45           |                                      |
| (P-3) 50% Mn+50% Al..... | 91  | 3.6                     | -0.42           |                                      |
| (P-3) 50% Mn+50% Al..... | 95+ | 3.95                    | -0.027          |                                      |

As can be seen from the foregoing Table IV densities above about 95% of the maximum density are to be avoided since the solution rate drops drastically at such high densities. The preferred densities for the compacted addition agent of the present invention are from about 65 to 90% of the maximum theoretical density.

The effect of initial particle sizing of the constituent materials on the solution rate for the addition agent of the present invention was also investigated using 50% Mn+50% Al compacts (1/8", 34 grams) having a density of about  $3.50 \pm 0.05$  g./cc. The results are shown in Table V.

TABLE V

Solution rate at 760° C., K aluminum size

| Manganese size | 20 mesh | 20 x 65 mesh | 150 mesh |
|----------------|---------|--------------|----------|
| 20 mesh.....   | -0.069  | -0.313       |          |
| 65 mesh.....   |         | -0.465       |          |
| 150 mesh.....  |         |              | -0.63    |

It has been found that for optimum results the sizing of the principal material and the promoter material should be substantially all finer than 20 mesh for optimum solubility in molten metal baths and preferably substantially all finer than 65 mesh.

It has been further found that the physical dimensions of the compacted addition agents of the present invention have an effect on the solution rate and it is preferred, when using pressed mixtures, that the compacts have one dimen-

sion not more than about  $\frac{1}{8}$  inch, and for optimum results not more than about  $\frac{1}{2}$  inch. That is to say, for example, with cylindrical compacts, either the diameter or length is preferably not more than about  $\frac{1}{8}$  inch; the optimum minimum dimension being from about  $\frac{1}{4}$  to  $\frac{1}{2}$  inch.

Table VI shows the solution rates obtained for different sized cylindrical compacts (density=3.40 $\pm$ 0.15 g./cc.) formed from electrolytic manganese (sized 150 MXD) and elemental aluminum (sized -100+325 mesh).

Table VI.—Effect of compact size

| Compact size (50% Mn+50% Al)<br>minimum dimension— <u>inches</u> : | Solution rate, K,<br>at 760° C. |
|--------------------------------------------------------------------|---------------------------------|
| $\frac{1}{4}$                                                      | -0.71                           |
| $\frac{1}{2}$                                                      | -0.64                           |
| $\frac{3}{4}$                                                      | -0.55                           |
| $\frac{7}{8}$                                                      | -0.30                           |

While the foregoing description has particularly described the making of principal material additions to molten aluminum baths, the additions of the present invention can be made to any metal bath in which the principal material is soluble. Such baths include aluminum, titanium, iron, and copper. The mesh sizes referred to herein are United States Sieve Series.

What is claimed is:

1. A process for making metal additions to a molten aluminum bath which comprises introducing into the molten aluminum bath a blended mixture consisting essentially of from about 10% to about 90% of finely divided aluminum and from about 10% to about 90% of at least one finely divided material selected from the group consisting of Mn, Cr, W, Mo, Ti, V, Fe, Co, Cu, Ni, Cb, Ta, Zr, Hf, Ag, and alloys thereof wherein the metal addition mixture is substantially all dissolved in the molten aluminum bath at an accelerated rate substantially greater than that which would be obtained with alloyed material of the same constituents and with substantially complete retention of the metal addition constituents.

2. A process in accordance with claim 1 wherein the blended mixture is in the form of compacts having a density of from about 65 to 95% of maximum theoretical density.

3. A process in accordance with claim 1 wherein the blended mixture is in the form of compacts having a density of from about 65 to 95% of maximum theoretical density and wherein the initial particle sizing of the blended mixture is substantially all finer than 20 mesh.

4. A process in accordance with claim 1 wherein the blended mixture is in the form of a compact having a density of from 65% to 95% of maximum theoretical density, wherein the initial particle sizing of the blended mixture is substantially all finer than 20 mesh and wherein such compacts have a maximum thickness of not more than about  $\frac{1}{8}$  inch.

5. A process in accordance with claim 1 wherein the blended mixture contains from about 10% to 90% aluminum and from about 10% to 90% manganese.

6. A process in accordance with claim 1 wherein the blended mixture contains from about 10% to about 90% aluminum and from about 10% to about 90% chromium.

7. A process in accordance with claim 1 wherein the blended mixture contains from about 10% to about 90% aluminum and from about 10% to about 90% ferromanganese.

8. A process in accordance with claim 1 wherein the blended mixture contains from about 10% to about 90% aluminum and from about 10% to about 90% ferrochromium.

9. A process for adding metal additions to a molten aluminum bath which comprises adding to the molten aluminum bath a mixture consisting essentially of from about 10 to about 90% of finely divided aluminum and from about 10 to about 90% of at least one finely divided material selected from the group consisting of manganese, tungsten, molybdenum, chromium, ferrochromium and ferromanganese wherein the metal addition mixture is substantially all dissolved in the molten aluminum bath at an accelerated rate substantially greater than that which would be obtained with alloyed material of the same constituents and with substantially complete retention of the metal addition constituents.

10. A process for making metal additions to a molten aluminum bath which comprises introducing into the molten aluminum bath a blended mixture consisting essentially of from about 10% to about 90% of finely divided aluminum and from about 10 to about 90% of at least one finely divided material selected from the group consisting of Mn, Cr, W, Mo, Ti, V, Fe, Co, Cu, Ni, Cb, Ta, Zr, Hf, Ag, and alloys thereof wherein upon introduction into the molten aluminum bath the aluminum coats with the selected material and the metal addition mixture is substantially all dissolved in the molten aluminum bath at an accelerated rate substantially greater than that which would be obtained with alloyed material of the same constituents and with substantially complete retention of the metal addition constituents.

11. A process in accordance with claim 1 wherein the blended mixture contains from about 20% to about 80% of finely divided aluminum and from about 20% to about 80% of at least one finely divided material selected from the group consisting of Mn, Cr, W, Mo, Ti, V, Fe, Co, Cu, Ni, Cb, Ta, Zr, Hf, Ag, and alloys thereof.

#### References Cited

#### UNITED STATES PATENTS

|    |           |        |                       |        |
|----|-----------|--------|-----------------------|--------|
| 50 | 2,935,397 | 5/1960 | Saunders et al. ----- | 75—129 |
|    | 3,190,750 | 6/1965 | Staggers et al. ----- | 75—138 |
|    | 3,459,540 | 8/1969 | Tisdale et al. -----  | 75—129 |

RICHARD O. DEAN, Primary Examiner

U.S. Cl. X.R.

75—129, 139, 143, 148, 160, 162, 175.5

UNITED STATES PATENT OFFICE  
CERTIFICATE OF CORRECTION

Patent No. 3,592,637 Dated July 13, 1971

Inventor(s) Charles M. Brown, Nicholas J. Pappas and Harry J. Brown

It is certified that error appears in the above-identified patent  
and that said Letters Patent are hereby corrected as shown below:

In column 2 at line 60 delete "Principal" and  
substitute ---Promoter---.

Signed and sealed this 29th day of February 1972.

(SEAL)  
Attest:

EDWARD M. FLETCHER, JR.  
Attesting Officer

ROBERT GOTTSCHALK  
Commissioner of Patents